

3,166,409  
SILICON-NIOBIUM ALLOYS

Roger Thomas John Hubbard, Sutton Coldfield, England, assignor to Imperial Metal Industries (Kynoch) Limited, London, England, a corporation of Great Britain No Drawing. Filed May 31, 1963, Ser. No. 284,378  
Claims priority, application Great Britain, June 1, 1962, 21,195/62

5 Claims. (Cl. 75—134)

This invention relates to niobium alloys. It is especially concerned with oxidation resistant alloys.

There are niobium alloys which retain their mechanical properties at high temperatures, but they are not resistant to oxidation. The most oxidation resistant strong niobium alloys are at least ten times more resistant to oxidation than pure niobium, but their oxidation rates are still about fifty times higher than could be tolerated in service.

Those niobium alloys which have sufficiently low oxidation rates are generally based on brittle intermetallic compounds. However, most of these alloys oxidise more rapidly at intermediate temperatures than at high temperatures, producing a low temperature oxidation rate peak. This peak may be shown by isothermal and slow thermal cyclic testing, both of which conditions may be encountered in service.

One of the most oxidation resistant binary intermetallic compounds of niobium in the disilicide  $\text{NbSi}_2$ , which is fairly resistant to high temperature oxidation but suffers from an oxidation rate peak at 1000—1050° C.

One object of the present invention is to improve the high temperature oxidation resistance and to reduce the oxidation rate peak of niobium disilicide by ternary alloying additions.

Accordingly the present invention provides alloys based on the intermetallic compound niobium disilicide, in which part of the niobium is replaced by at least one of the metals aluminum, chromium, iron or titanium, these addition elements being present in such amounts as to maintain the disilicide stoichiometry of the compound. Thus the alloys of the present invention are of the composition represented by the formula  $\text{MSi}_2$  where M is niobium plus at least one of the addition elements listed, to a total of 33½ atomic percent. The silicon content is always about 66½ atomic percent and preferably does not vary by more than plus or minus two atomic percent.

We have found that such alloys possess high oxidation resistance both at elevated temperatures and at lower temperatures and are resistant to oxidation during cycles of heating and cooling, especially after a high temperature oxide film has been formed.

We have found that small additions of the metals listed are effective and that the improvement in properties is maintained when over half of the niobium has been replaced. In particular we have found that up to 23½ atomic percent of the addition elements reduces the rate of oxidation. Although some improvement in oxidation resistance is obtained over the whole range there are certain limitations to the amounts of addition for optimum beneficial effect. Alloys containing aluminum in excess of about 10% have low melting point constituents which are exuded on the surface at high temperatures. Alloys containing less than about 6½ atomic percent titanium deteriorate due to severe oxidation and thickening of the scale which spalls on cooling.

Preferred ranges of composition are up to 10 and preferably 1½ to 6½ atomic percent aluminium, 1½ to 23½ atomic percent chromium, 1½ to 23½ atomic percent iron and from 6½ to 23½ atomic percent titanium.

Properties of certain alloys exemplifying the invention are listed in the accompanying table.

All the alloys exemplified are based on the intermetallic compound niobium disilicide containing 33½ atomic percent niobium and 66½ atomic percent silicon. The composition of the alloys is of the general form  $\text{MSi}_2$  where M represents niobium plus one of the addition elements aluminum, chromium, iron, titanium, the total atomic percentage of M being 33½. For comparison, results are also given for niobium disilicide without addition.

Test 1 was performed as follows:

- (a) Clean samples—as cast and ground to a rectangular block.
- 15 (b) Heated from 600° C. to 1200° C. at 6° C./min.
- (c) Held at 1200° C. for 30 min.
- (d) Cooled from 1200° C. to 600° C. in 60 min.
- (e) Total duration of test—about 200 min.
- 20 (f) Results expressed as weight gain of sample during complete test per unit surface area per hour (mg./sq. cm./hr.).

This test indicates the formation of an initial high temperature oxide film on the surface. After the film has been formed the rate of oxidation is reduced.

Test 2 was performed as follows:

- (a) Samples from Test 1 (i.e., with an adherent oxide film present).
- 30 (b) Heated for 24 hours at 1200° C.
- (c) Results expressed as weight gain per unit surface area per hour (mg./sq. cm./hr.).

This test was designed to show the oxidation rate at a constant temperature of 1200° C. after an initial oxide film has been formed.

Test 3 was performed as follows:

- (a) Samples from Test 2.
- (b) Heated at 1200° C. for 15 min.
- 40 (c) Cooled to 600° C. in 60 min.
- (d) Heated from 600° C. to 1200° C. at 6° C./min.
- (e) Results expressed as in Test 1(f).

This test shows the behaviour on heating and cooling and is the most significant test, since it indicates the resistance to oxidation over a range of temperatures under conditions of heating and cooling typical of those encountered in service.

Test 4 was performed as follows:

- 50 (a) Samples from Test 3.
- (b) Heated for 100 hrs. at 1100° C.
- (c) Results expressed as in Test 2(c).

This test shows the long-term oxidation characteristics including the effect of oxygen contamination, the possibility of the oxide film spalling off if it becomes too thick, and the presence of low melting point constituents.

It will be seen from the results that all the alloys listed are more resistant to oxidation than niobium disilicide. 60 The rate of oxidation of niobium disilicide itself is less than that of niobium by a factor of about 50. The properties revealed by Test 3 are particularly significant.

Alloys containing more than 10 atomic percent of aluminium contain low melting point phases which were 65 exuded as globules on the surface during oxidation at 1100° C. and 1200° C. Alloys containing 3½ and 6½ atomic percent chromium formed an oxide film which spalled on cooling to room temperature. Alloys containing up to 6½ atomic percent of titanium suffered from 70 spalling of the oxide scale.

The alloys of the present invention are brittle and diffi-

cult to fabricate but they can be employed in the cast form or used as oxidation resistant coatings on other niobium alloys.

4. A niobium-silicon alloy consisting essentially of 64 $\frac{1}{3}$  to 68 $\frac{1}{3}$  atomic percent silicon, 1 $\frac{1}{3}$  to 23 $\frac{1}{3}$  atomic percent iron and the balance niobium.

| Addition element | Atomic percent   |                  |                            | Test 1 | Test 2 | Test 3 | Test 4 | Condition of film |
|------------------|------------------|------------------|----------------------------|--------|--------|--------|--------|-------------------|
|                  | Nb $\pm 1\%$     | Si $\pm 2\%$     | Addition element $\pm 1\%$ |        |        |        |        |                   |
| Al               | 31 $\frac{1}{3}$ | 66 $\frac{2}{3}$ | 1 $\frac{1}{3}$            | 0.11   | 0.019  | N      | N      | VG                |
|                  | 30               | 66 $\frac{2}{3}$ | 3 $\frac{1}{3}$            | 0.12   | N      | N      | 0.014  | VG                |
|                  | 28 $\frac{1}{3}$ | 66 $\frac{2}{3}$ | 6 $\frac{1}{3}$            | 0.11   | 0.03   | 0.03   | 0.014  | GL                |
| Cr               | 31 $\frac{1}{3}$ | 66 $\frac{2}{3}$ | 1 $\frac{1}{3}$            | 0.10   | 0.014  | 0.06   | 0.015  | GL                |
|                  | 30               | 66 $\frac{2}{3}$ | 3 $\frac{1}{3}$            | 0.22   | 0.03   | 0.10   | -----  | SL                |
|                  | 26 $\frac{1}{3}$ | 66 $\frac{2}{3}$ | 6 $\frac{1}{3}$            | 0.12   | N      | N      | 0.03   | SL                |
|                  | 23 $\frac{1}{3}$ | 66 $\frac{2}{3}$ | 10                         | 0.17   | 0.05   | N      | 0.003  | VG                |
|                  | 16 $\frac{1}{3}$ | 66 $\frac{2}{3}$ | 16 $\frac{2}{3}$           | 0.21   | 0.05   | 0.09   | 0.002  | VG                |
|                  | 10               | 66 $\frac{2}{3}$ | 23 $\frac{1}{3}$           | 0.35   | 0.076  | 0.04   | 0.022  | S <sub>2</sub>    |
| Fe               | 31 $\frac{1}{3}$ | 66 $\frac{2}{3}$ | 1 $\frac{1}{3}$            | 0.30   | N      | N      | -----  | VG                |
|                  | 30               | 66 $\frac{2}{3}$ | 3 $\frac{1}{3}$            | 0.48   | N      | N      | 0.001  | GL                |
|                  | 26 $\frac{1}{3}$ | 66 $\frac{2}{3}$ | 6 $\frac{1}{3}$            | 0.29   | N      | 0.06   | 0.001  | GL                |
|                  | 23 $\frac{1}{3}$ | 66 $\frac{2}{3}$ | 10                         | 0.35   | 0.03   | 0.02   | 0.008  | GL                |
|                  | 16 $\frac{1}{3}$ | 66 $\frac{2}{3}$ | 16 $\frac{2}{3}$           | 0.17   | 0.03   | 0.02   | N      | GL                |
|                  | 10               | 66 $\frac{2}{3}$ | 23 $\frac{1}{3}$           | 0.30   | 0.022  | 0.022  | 0.004  | F                 |
| Ti               | 26 $\frac{1}{3}$ | 66 $\frac{2}{3}$ | 6 $\frac{1}{3}$            | 0.11   | 0.01   | 0.07   | 0.08   | S <sub>1</sub>    |
|                  | 23 $\frac{1}{3}$ | 66 $\frac{2}{3}$ | 10                         | 0.13   | 0.01   | 0.02   | 0.003  | GL                |
|                  | 16 $\frac{1}{3}$ | 66 $\frac{2}{3}$ | 16 $\frac{2}{3}$           | 0.18   | 0.02   | 0.09   | N      | VG                |
|                  | 10               | 66 $\frac{2}{3}$ | 23 $\frac{1}{3}$           | 0.08   | 0.034  | N      | N      | F                 |
|                  | -----            | 66 $\frac{2}{3}$ | 33 $\frac{1}{3}$           | N      | -----  | -----  | -----  | F                 |
| —                | 33 $\frac{1}{3}$ | 66 $\frac{2}{3}$ | -----                      | 0.65   | 0.25   | 0.48   | -----  | S <sub>1</sub>    |

N=Negligible oxidation, weight gain less than 0.1 mg./cm.<sup>2</sup> during test.

Condition of Film—

VG=Very good adherent uniform film.

SL=Film spalled in places due to localised oxidation.

GL=Good film, but some slight localised oxidation due to inhomogeneity.

F=Glassy film of silica or silicate.

S<sub>1</sub>=Severe spalling on cooling to room temperature.

S<sub>2</sub>=Slight spalling.

I claim:

1. A niobium-silicon alloy consisting essentially of: 64 $\frac{1}{3}$  to 68 $\frac{1}{3}$  atomic percent silicon, an addition agent selected from the group consisting of 1 $\frac{1}{3}$  to 10 atomic aluminum, 1 $\frac{1}{3}$  to 23 $\frac{1}{3}$  atomic percent chromium, 1 $\frac{1}{3}$  to 23 $\frac{1}{3}$  atomic percent iron and 6 $\frac{1}{3}$  to 23 $\frac{1}{3}$  atomic percent titanium, and the balance essentially niobium. 40

2. A niobium-silicon alloy consisting essentially of 64 $\frac{1}{3}$  to 68 $\frac{1}{3}$  atomic percent silicon, 1 $\frac{1}{3}$  to 10 atomic percent aluminum and the balance niobium.

3. A niobium-silicon alloy consisting essentially of 64 $\frac{1}{3}$  to 68 $\frac{1}{3}$  atomic percent silicon, 1 $\frac{1}{3}$  to 23 $\frac{1}{3}$  atomic percent chromium and the balance niobium.

35 5. A niobium-silicon alloy consisting essentially of 64 $\frac{1}{3}$  to 68 $\frac{1}{3}$  atomic percent silicon, 6 $\frac{1}{3}$  to 23 $\frac{1}{3}$  atomic percent titanium and the balance niobium.

#### References Cited by the Examiner

#### UNITED STATES PATENTS

2,169,193 8/39 Comstock ----- 75—134.3  
2,939,785 6/60 Weatherly et al. ----- 75—174

45 DAVID L. RECK, Primary Examiner.

WINSTON A. DOUGLAS, Examiner,